

## UNITED STATES PATENT OFFICE

HARRY P. BASSETT, OF CYNTHIANA, KENTUCKY, AND THOMAS F. BANIGAN, OF CLIFTON HEIGHTS, PENNSYLVANIA, ASSIGNEES, BY MESNE ASSIGNMENTS, TO MEIGS, BASSETT & SLAUGHTER, INC., OF PHILADELPHIA, PENNSYLVANIA, A CORPORATION OF PENNSYLVANIA

## PROCESS OF MERCERIZING

No Drawing.

Application filed January 30, 1925. Serial No. 5,887.

This invention relates to processes of mercerizing and particularly mercerizing woven and unwoven natural cellulose fibres such as cotton and linen having interwoven therewith artificial filaments commonly known as 5 artificial silk, although our invention is adapted for advantageous use in mercerizing natural cellulose fibres unassociated with artificial silk filaments.

Heretofore it has been proposed to 10 protect artificial silk filaments of viscose silk interwoven with natural cellulose fibres from the deleterious action of the mercerizing solution by the addition to such solution of 15 so-called caustic alkali modifying agents intended to prevent such deleterious action, but such processes have so far as we have been able to learn, not come into commercial use and, from our experiments, they appear 20 to be incapable of successful practical use.

In the operation of our process, we recognize two individual types of artificial silk; first, silk consisting essentially of pure cellulose including viscose, and second, cellulose 25 ester silks consisting of cellulose in combination with organic acids. The term "cellulose containing materials" as herein employed includes both of these types of artificial silk as well as natural cellulose fibres.

We have discovered that artificial 30 filaments of cellulose silk or artificial filaments of cellulose esters intermingled or interwoven with natural cellulose fibres cannot be protected from deleterious action of caustic alkali mercerizing solution in the mercerizing process by the mere use in the mercerizing bath of a so-called caustic alkali modifying agent capable of repressing the tendency 35 of the caustic alkali to decompose the artificial silk in the mercerizing solution and thereby injure the quality of the artificial cellulose filaments or cellulose ester filaments during the mercerizing process. Protection in the initial step of mercerizing can be obtained by introducing the intermingled or 40 interwoven fibres or filaments free of water or of water of weak solutions into the mercerizing solution containing, in addition to the caustic alkali, an agent capable of substantially 45 repressing the tendency of the

caustic alkali to ionize and consequently the tendency of the artificial cellulose or the cellulose ester to decompose in the mercerizing solution.

By the expression "free of water" as used herein, we refer to water as such, that is, containing no substantially free and uncombined water, as distinguished from a solution of a salt wherein the solution is substantially saturated with a salt and accordingly incapable 55 of performing or acting as water or weak solutions of salts in the practice of our process.

We have also discovered that cellulose esters whenever exposed to the action of caustic alkali solution of sufficient concentration to 60 effect any mercerization of cellulose are injured and their quality impaired unless such caustic alkali solution is modified by the presence of a protective material capable of counteracting or repressing the tendency of the 65 caustic alkali to ionize in solution and consequently capable of repressing the tendency of the cellulose ester to decompose when in contact with such caustic alkali solution under the conditions ordinarily employed in the 70 process of mercerization.

We have found that when the caustic alkali solution containing the modifying agent is 75 washed from the material being treated with water the ionization resulting from the reduction of the concentration of solution of salts remaining in the fibres materially injures the artificial silk filaments and causes them to assume a ropey or gelatinous consistency and when under tension deprives 80 them of lustre as well as weakening their strength. Thus the use of sodium acetate and similar salts as a modifying agent only in the mercerizing bath becomes practically ineffective and renders the process inoperative 85 unless the artificial silk fibres are protected during the washing operation. We therefore proceed as follows: After the mercerizing treatment is completed the process 90 is continued by washing the mercerizing solution from the treated fibres by using a substantially saturated solution of the agent employed to repress the tendency of the caustic alkali to ionize and the artificial silk to de- 95 100

compose, until the concentration of the caustic alkali solution left in the fibres has been reduced below the concentration at which mercerization of the cellulose or decomposition of the artificial silk can occur.

5 Thereafter the material is washed substantially free of the solution of such agent and finally bleaching, dyeing or finishing the textile may be carried out in any suitable manner.

10 We also have discovered that artificial cellulose filaments and natural cellulose fibres are injuriously affected whenever they are exposed to the action of strong caustic alkali 15 solution unless the alkali solution is suitably modified to repress the ionization of the caustic alkali. Greater lustre and softness are obtained when the fibres and filaments are protected against the harmful effect of ionization 20 of the caustic alkali solution at all stages of the mercerizing process when the fibres and filaments are in contact with alkali solution having sufficient concentration to produce mercerization of cellulose as well as 25 when the fibres and filaments are protected against the action of the caustic alkali only to the extent of modifying the mercerizing solution itself.

30 The natural cellulose fibres, cellulose ester filaments, artificial cellulose filaments, or mixtures of the same, may be introduced dry into the mixed mercerizing bath but we prefer to wet the fibres and filaments before introducing them into the mercerizing solution with 35 a substantially concentrated solution of the agent employed to repress the decomposition of the artificial cellulose material and the ionization of the caustic alkali in the mercerizing bath.

40 We have found that sodium acetate is preferably and usually superior to all other agents for repressing the decomposition of the cellulose esters in the mercerizing bath, which we have investigated and we prefer to make 45 use of this salt in the practice of our process.

50 We have also discovered that not only are filaments of cellulose esters and artificial cellulose filaments injuriously affected by the action of caustic alkali in mercerization with 55 an unmodified mercerizing solution, but that natural cellulose fibres and particularly woven cotton fibres have a stiff and harsh feeling after mercerization by the ordinary method of mercerization, their flexibility and softness having been impaired. We have discovered also that this injurious effect of the mercerizing 60 solution is prevented by the use of sodium acetate as described in connection with the treatment of intermingled and interwoven natural cellulose fibres, cellulose ester filaments, and artificial cellulose filaments.

65 In the preferred practice of our process, the natural cellulose fibres or such fibres intermingled or interwoven with artificial cellulose filaments or cellulose ester filaments, or

mixtures of the same, either loose, in thread or in yarn, or woven into fabric, are first moistened and preferably thoroughly wet with a substantially saturated solution of sodium acetate, then subjected to the well known mercerizing process in a bath containing in addition to the caustic alkali, sodium acetate in substantially saturated solution therein. The treated material is then washed substantially free of caustic alkali 70 with a substantially concentrated solution of sodium acetate and such material washed substantially free of sodium acetate solution with water. The washed material is finally dyed, bleached, or finished in any suitable 75 manner.

If some agent other than sodium acetate such as heretofore has been suggested for the protection of filaments or viscose silk, is employed to repress the tendency of the cellulose containing fibres or filaments to decompose in the mercerizing solution a concentrated solution of such agent should preferably be used in the pretreatment described although as above indicated such fibres or 85 filaments or both may be introduced dry into the mercerizing bath, and a substantially saturated solution of such protective agent should be employed in washing the treated 90 fibres or filaments substantially free of the caustic alkali.

Having described our invention, we claim:

1. The process of treating cellulose textiles and the like, containing artificial silk filaments, which comprises introducing said material into a caustic alkali mercerizing solution containing a salt which has an organic base and will not by reaction of the caustic alkali therewith undergo change in its chemical composition, removing said material from 100 said mercerizing solution and then washing with a solution of said salt until the concentration of the caustic alkali has been reduced below that at which mercerization takes place.

2. The process of treating cellulose textiles and the like, containing artificial silk filaments, which comprises introducing said material into a caustic alkali mercerizing solution containing sodium acetate, mercerizing the natural cellulose fibres therein, removing said material from said mercerizing solution and then washing with sodium acetate until the concentration of the caustic alkali in the fibres and filaments has been reduced below that at which mercerization 115 takes place.

3. The process of treating cellulose textiles and the like, containing artificial silk filaments, which comprises introducing said material into a caustic alkali mercerizing solution, containing a salt which has an organic base and will not by reaction of the caustic alkali therewith undergo change in its chemical composition, removing said material from 125 said mercerizing solution, washing with a 130

solution of said salt until the concentration of the caustic alkali has been reduced below that at which mercerization takes place, and then washing with water until substantially free from said last named salt.

5 4. The process of treating cellulose textiles and the like, containing artificial silk filaments, which comprises introducing said material into a caustic alkali mercerizing solution, containing sodium acetate, mercerizing the natural cellulose fibres therein, removing said material from said mercerizing solution, washing with sodium acetate until the concentration of the caustic alkali in the 10 fibres and filaments has been reduced below that at which mercerization takes place, and then washing with water until substantially free from said last named sodium acetate.

15 5. A process of mercerizing textiles and the like which include natural cellulose fibres that may have intermingled or interwoven therewith artificial cellulose filaments, or mixtures of the same, the steps comprising, first wetting the material with a substantially 20 saturated solution of sodium acetate, then introducing the thus treated material into a mercerizing bath containing in addition to caustic alkali, sodium acetate in substantially saturated solution therein, subjecting the material to the mercerizing process therein, washing the treated material substantially free of caustic alkali with a substantially saturated solution of sodium acetate, and washing such material substantially free of sodium 25 acetate solution.

30 6. A process of mercerizing textiles and the like which include natural cellulose fibres that may have intermingled or interwoven therewith artificial cellulose filaments, cellulose ester filaments, or mixtures of the same, the steps, comprising, introducing the material into a mercerizing bath containing in addition to caustic alkali, sodium acetate in substantially saturated solution therein, 35 washing the treated material substantially free of caustic alkali with a substantially saturated solution of sodium acetate, and washing such material substantially free of sodium acetate solution.

40 7. A process of mercerizing textiles and the like which include natural cellulose fibres that may have intermingled or interwoven therewith artificial cellulose filaments, cellulose ester filaments, or mixtures of the same, the steps, comprising, first wetting the material with a substantially saturated solution of an agent for protecting cellulosic fibres and filaments from the injurious action of 45 caustic soda, such agent being a material capable of repressing the ionization of caustic alkali and of repressing the decomposition of cellulose ester filaments in contact with the caustic alkali mercerizing solution, subjecting 50 the thus treated material to the mercerizing

process in a bath containing in addition to caustic alkali, such ionization repressing agent in substantially saturated solution therein, washing the treated material substantially free of caustic alkali with a substantially saturated solution of such ionization repressing agent, and washing the material substantially free of the solution of such agent.

55 8. A process of mercerizing textiles and the like which include natural cellulose fibres that may have intermingled or interwoven therewith artificial cellulose filaments, cellulose ester filaments, or mixtures of the same, the steps, comprising, introducing the material into a mercerizing bath containing in addition to the caustic alkali an agent for repressing the ionization of caustic alkali and repressing the decomposition of cellulose ester filaments in contact with the caustic alkali mercerizing solution, subjecting the material to the mercerizing process in such bath, washing the treated material substantially free of caustic alkali with a substantially saturated solution of such ionization repressing 60 agent, and washing the material substantially free of the solution of such agent.

85 9. In the process of mercerizing natural cellulose fibres having intermingled or interwoven therewith cellulose acetate filaments, the steps of subjecting such fibres and filaments to the mercerizing action of a caustic alkali mercerizing solution containing sodium acetate in substantially saturated solution 90 therein, removing said fibres and filaments from said mercerizing solution, and then washing with a solution of said salt until the concentration of the caustic alkali has been reduced below that at which mercerization 95 takes place.

100 10. In the process of mercerizing natural cellulose fibres having intermingled or interwoven therewith cellulose acetate filaments, the step of subjecting such fibers and filaments substantially free of water to the mercerizing action of a caustic alkali mercerizing solution containing sodium acetate in substantially saturated solution 105 therein.

110 11. In the process of mercerizing substantially water-free intermingled or interwoven natural cellulose fibers and cellulose acetate by the action of a caustic alkali mercerizing solution, protecting the cellulose acetate filaments from the injurious action of the caustic alkali therein during the mercerizing process by the action of sodium acetate in substantially saturated solution in said mercerizing solution.

115 12. In the process of mercerizing substantially water-free intermingled or interwoven cellulose fibers and cellulose acetate by the action of a caustic alkali mercerizing solution, protecting the cellulose acetate filaments from the injurious action of the caustic alkali 120 125 130

therein by the action of an acetate freely soluble in the mercerizing solution and in substantially saturated solution in such mercerizing solution.

5 In testimony whereof we affix our signatures.

**HARRY P. BASSETT.**  
**THOMAS F. BANIGAN.**

**10****15****20****25****30****35****40****45****50****55****60****65**